

# UNITED STATES PATENT OFFICE.

LOUIS COLLARDON, OF LEIPZIG, GERMANY

## PROCESS OF MANUFACTURING PRINTING BLOCKS AND PLATES.

No. 851,918.

Specification of Letters Patent.

Patented April 30, 1907.

Application filed January 23, 1905. Serial No. 242,452.

To all whom it may concern:

Be it known that I, LOUIS COLLARDON, retired military officer, manufacturer, a citizen of the Argentine Republic, residing at 32 Friedrich Liststrasse, Leipzig, Kingdom of Saxony, German Empire, have invented new and useful Improvements in Process of Manufacturing Printing Blocks and Plates, of which the following is a specification.

10 This invention relates to a new sort of printing plates and the manufacture of them and has for its object to render the printing plates cheaper and more durable and the process of the manufacture cheaper and 15 more expeditious.

The printing plates according to my invention are especially capable for reproducing fine details. They have furthermore the 20 advantage to be practically nearly uninflammable, which is important, because printing blocks or plates are generally cleaned by washing with benzene, solvent naphtha etc., in order to remove the remainder of the colors, in which operation easily inflammation 25 can happen.

The printing plates according to my invention consist of hardened casein or albumen. The process of hardening casein or albumen may be carried out by means of 30 substances as tanning substances, formic aldehyde, hexamethylenetetramine, bichromates, chromates, etc. the hardening action of which on casein or albumen is known. The process of manufacturing printing plates 35 can be carried out in the following manner: I take finely powdered insoluble casein and moisten the casein with a moistening medium of neutral character, as water for example, or with a moistening medium of acid or alkaline reaction. For instance highly concentrated liquid ammonia may be employed and of such a quantity that a complete solution of the casein does not take place. The quantity of the moistening medium must be such 45 that the mass still feels dry comparatively, so that but very small quantities of liquid are present.

The moistened casein is placed into a mold of suitable, for instance quadrangular, shape 50 and is then exposed to a high pressure, during or after which a heating can take place, by conducting heat to the surface of the mold or into the interior of it. The mold can be provided with a steam jacket or such like. 55 The measure of the high pressure and of the

temperature used may be found by the skilled workman by experiments. After the treatment by pressure and heat the plates are allowed to cool and are then hardened by being coated with hardening means, the action of which may be assisted by warming the plates. I may however also with preference manufacture printing plates being hardened not only on their surface but throughout their whole mass. I mix the 65 casein with the hardening agents before moistening, moisten then, place the mass into the mold and apply heat and pressure. When hexamethylenetetramine which has proved to be particularly suitable, is employed as hardening agent, it is advantageous to add to casein a substance, such as an acid, producing an acid reaction, as the separation of formaldehyde from hexamethylenetetramine is facilitated. As many tannins 70 have an alkaline reaction and the hardening of the casein is then less efficient, substances presenting an acid reaction are added in this case also. Among acid substances, which may be added to the casein, in addition to 75 acids generally, solid acids or acid salts, such for example as dicalciumphosphate and generally acid phosphates, borates or chromates may be employed, also Turkey-red oil, organic acids such as oleic acid, stearic acid 80 and their salts. The amount of such additions will be ascertained by the skilled workman by experiments and will be suitably 10 percent of the casein used.

For many purposes hardened casein or albumen is not of itself sufficiently durable and it is very desirable to produce a greater degree of hardness. In other cases, again it is necessary to make the plates softer.

In some cases it is suitable to modify the 95 hardness of the printing plates obtained by my process of producing hard casein or albumen plates.

In order to obtain more softness the plates are brought into contact with an appropriate 100 oil, such for example as castor oil, Canada balsam, Turkey-red oil, turpentine and the like. Soft filling material such as sulfate of barium, magnesia, chalk, permanent white, white lead, kaolin or the like may be employed.

The printing plates obtained according to my invention may be used as printing surfaces for lithographic printing or for relief-printing. If one intends to use the plates for 110

lithographic printing, one transfers the picture on the printing plate in the same manner as usual in the lithographic art.

In order to produce a matrix from my hardened casein plates, I may proceed in the following way: A hardened plate of casein or albumen polished on one side is placed upon a hot place, or heated on a paraffin bath or the like to say 80 to 90° C. Upon the plate, 5 which has thus been made plastic, is then placed an engraved or etched die, also heated and applied with a suitable pressure in the heated condition and cooling is then allowed to take place under pressure. The skilled 10 workman will find by experiments the pressure required for obtaining a clean sharp copy suitable for his special purposes.

From the matrix obtained in the described manner I can prepare copies by placing the 20 matrix on a heated hardened casein plate, softer than the plate from which the matrix has been made, and applying pressure to the said plates. The copy thus obtained can be used for printing in letter presses etc.

25 What I claim as my invention, and desire to secure by Letters Patent is:

1. The process of manufacturing printing

blocks and plates which consists in moistening insoluble casein in form of a very fine powder and mixing the same with a hardening medium throughout its entire mass and submitting it to pressure and heat substantially as described. 30

2. The process of manufacturing printing blocks and plates which consists in moistening the casein with a small quantity of ammonia, mixing it with hexamethylentetramine and submitting it to pressure and heat, substantially as described. 35

3. The process of manufacturing printing blocks and plates which consists in moistening insoluble casein mixing the same with a hardening medium and substances modifying the hardness throughout its entire mass and submitting it to pressure and heat substantially as described. 40

In testimony whereof I have signed my name to this specification in the presence of two subscribing witnesses.

LOUIS COLLARDON.

Witnesses:

WOLDEMAR HAUPT,  
HENRY HASPER.